



US005805964A

**United States Patent** [19]**Badesha et al.****Patent Number:** **5,805,964****Date of Patent:** **Sep. 8, 1998**[54] **INORGANIC COATED DEVELOPMENT ELECTRODES AND METHODS THEREOF**

[75] Inventors: **Santokh S. Badesha; Arnold W. Henry**, both of Pittsford; **George J. Heeks; J. Stephen Kittelberger**, both of Rochester; **John G. VanDusen, Walworth; Suresh K. Ahuja, Webster; Merlin E. Scharfe, Penfield; Richard L. Schank, Pittsford; Mark J. Hirsch, Fairport**, all of N.Y.

[73] Assignee: **Xerox Corporation**, Stamford, Conn.[21] Appl. No.: **841,234**[22] Filed: **Apr. 29, 1997**[51] Int. Cl.<sup>6</sup> **G03G 15/06**[52] U.S. Cl. **399/266; 399/290**[58] Field of Search **399/266, 290, 399/291**[56] **References Cited**

## U.S. PATENT DOCUMENTS

4,868,600 9/1989 Hays et al. .... 355/259

|           |         |                        |          |
|-----------|---------|------------------------|----------|
| 4,984,019 | 1/1991  | Folkins .....          | 355/215  |
| 5,010,368 | 4/1991  | O'Brien .....          | 399/266  |
| 5,124,749 | 6/1992  | Bares .....            | 355/202  |
| 5,172,170 | 12/1992 | Hays et al. ....       | 355/259  |
| 5,270,782 | 12/1993 | Floyd, Jr. ....        | 399/266  |
| 5,300,339 | 4/1994  | Hays et al. ....       | 428/36.9 |
| 5,311,258 | 5/1994  | Brewington et al. .... | 399/266  |
| 5,448,342 | 9/1995  | Hays et al. ....       | 355/259  |

**OTHER PUBLICATIONS**

Xerox Disclosure Journal, vol. 14, No. 1, Jan./Feb. 1989 entitled "Metal Cleaning Blade with Diamond Coating", by Paul F. Morgan.

*Primary Examiner*—Arthur T. Grimley*Assistant Examiner*—Quana Grainger*Attorney, Agent, or Firm*—Annette L. Bade

[57]

**ABSTRACT**

An apparatus and process for reducing accumulation of toner from the surface of an electrode member in a development unit of an electrostatographic printing apparatus by providing an inorganic coating on at least a portion of the electrode member.

**20 Claims, 3 Drawing Sheets**



**FIG. 1**



FIG. 2



FIG. 3

**FIG. 4****FIG. 5** PRIOR ART

**INORGANIC COATED DEVELOPMENT  
ELECTRODES AND METHODS THEREOF**

**CROSS REFERENCE TO RELATED  
APPLICATIONS**

Attention is directed to the following copending applications assigned to the assignee of the present application: Attorney Docket No. D/96244, U.S. application Ser. No. 08/841,033 filed Apr. 29, 1997, entitled, "Coated Development Electrodes and Methods Thereof," Attorney Docket No. D/96244Q1, U.S. application Ser. No. 08/841,136 filed Apr. 29, 1997, entitled, "Organic Coated Development Electrodes and Methods Thereof," Attorney Docket No. D/96244Q3, U.S. application Ser. No. 08/841,034 filed Apr. 29, 1997, entitled, "Composite Coated Development Electrodes and Methods Thereof," and Attorney Docket No. D/96244Q4, U.S. application Ser. No. 08/841,235 filed Apr. 29, 1997, entitled "Coating Compositions for Development Electrodes and Methods Thereof." The disclosures of each of these applications are hereby incorporated by reference in their entirety.

**BACKGROUND OF THE INVENTION**

The present invention relates to methods, processes and apparatus for development of images, and more specifically, to electrode members for use in a developer unit in electro-photographic printing machines. Specifically, the present invention relates to methods and apparatus in which at least a portion of a development unit electrode member is coated with a coating material, and in embodiments, a low surface energy coating material. In embodiments, electrode member history, damping and/or toner accumulation is controlled or reduced.

Generally, the process of electrophotographic printing includes charging a photoconductive member to a substantially uniform potential so as to sensitize the photoconductive member thereof. The charged portion of the photoconductive member is exposed to a light image of an original document being reproduced. This records an electrostatic latent image on the photoconductive member. After the electrostatic latent image is recorded on the photoconductive member, the latent image is developed by bringing a developer material into contact therewith. Two component and single component developer materials are commonly used. A typical two component developer material comprises magnetic carrier granules having toner particles adhering triboelectrically thereto. A single component developer material typically comprises toner particles. Toner particles are attracted to the latent image forming a toner powder image on the photoconductive member. The toner powder image is subsequently transferred to a copy sheet. Finally, the toner powder image is heated to permanently fuse it to the copy sheet in image configuration.

One type of single component development system is a scavengerless development system that uses a donor roll for transporting charged toner to the development zone. At least one, and preferably a plurality of electrode members are closely spaced to the donor roll in the development zone. An AC voltage is applied to the electrode members forming a toner cloud in the development zone. The electrostatic fields generated by the latent image attract toner from the toner cloud to develop the latent image.

Another type of two component development system is a hybrid scavengerless development system which employs a magnetic brush developer roller for transporting carrier having toner adhering triboelectrically thereto. A donor roll

is used in this configuration also to transport charged toner to the development zone. The donor roll and magnetic roller are electrically biased relative to one another. Toner is attracted to the donor roll from the magnetic roll. The electrically biased electrode members detach the toner from the donor roll forming a toner powder cloud in the development zone, and the latent image attracts the toner particles thereto. In this way, the latent image recorded on the photoconductive member is developed with toner particles.

Various types of development systems have hereinbefore been used as illustrated by the following disclosures.

U.S. Pat. No. 4,868,600 to Hays et al., the subject matter of which is hereby incorporated by reference in its entirety, describes an apparatus wherein a donor roll transports toner to a region opposed from a surface on which a latent image is recorded. A pair of electrode members are positioned in the space between the latent image surface and the donor roll and are electrically biased to detach toner from the donor roll to form a toner cloud. Detached toner from the cloud develops the latent image.

U.S. Pat. No. 4,984,019, to Folkins, the subject matter of which is hereby incorporated by reference in its entirety, discloses a developer unit having a donor roll with electrode members disposed adjacent thereto in a development zone. A magnetic roller transports developer material to the donor roll. Toner particles are attracted from the magnetic roller to the donor roller. When the developer unit is inactivated, the electrode members are vibrated to remove contaminants therefrom.

U.S. Pat. No. 5,124,749 to Bares, the subject matter of which is hereby incorporated by reference in its entirety, discloses an apparatus in which a donor roll advances toner to an electrostatic latent image recorded on a photoconductive member wherein a plurality of electrode wires are positioned in the space between the donor roll and the photoconductive member. The wires are electrically biased to detach the toner from the donor roll so as to form a toner cloud in the space between the electrode wires and the photoconductive member. The powder cloud develops the latent image. A damping material is coated on a portion of the electrode wires at the position of attachment to the electrode supporting members for the purpose of damping vibration of the electrode wires.

U.S. Pat. Nos. 5,300,339 and 5,448,342 both to Hays et al., the subject matter each of which is hereby incorporated by reference in their entirety, disclose a coated toner transport roll containing a core with a coating thereover.

U.S. Pat. No. 5,172,170 to Hays et al., the subject matter of which is hereby incorporated by reference in its entirety, discloses an apparatus in which a donor roll advances toner to an electrostatic latent image recorded on a photoconductive member. The donor roll includes a dielectric layer disposed about the circumferential surface of the roll between adjacent grooves.

Primarily because the adhesion force of the toner particles is greater than the stripping force generated by the electric field of the electrode members in the development zone, a problem results in that toner tends to build up on the electrode members. Accumulation of toner particles on the wire member causes non-uniform development of the latent image, resulting in print defects. The problem is aggravated by toner fines and any toner components, such as high molecular weight, crosslinked and/or branched components, and the voltage breakdown between the wire member and the donor roll.

One specific example of toner contamination results upon development of a document having solid areas which require

a large concentration of toner to be deposited at a particular position on the latent image. The areas of the electrode member corresponding to the high throughput or high toner concentration areas tend to include higher or lower accumulation of toner because of this differing exposure to toner throughput. When the printer subsequently attempts to develop another, different image, the toner accumulation on the electrode member will lead to differential development of the newly developed image corresponding to the areas of greater or lesser toner accumulation on the electrode members. The result is a darkened or lightened band in the position corresponding to the solid area of the previous image. This is particularly evident in areas of intermediate density, since these are the areas most sensitive to differences in development. These particular image defects caused by toner accumulation on the electrode wires at the development zone are referred to as wire history. FIG. 5 contains an illustration of wire contamination and wire history. Wire contamination results when fused toner forms between the electrode member and donor member due to toner fines and any toner components, such as high molecular weight, crosslinked and/or branched components, and the voltage breakdown between the wire member and the donor roll. Wire history is a change in developability due to toner or toner components sticking to the top of the electrode member.

Accordingly, there is a specific need for electrode members in the development zone of a development unit of an electrophotographic printing machine which provide for a decreased tendency for toner accumulation in order to decrease wire history and wire contamination, especially at high throughput areas, and decreasing the production of unwanted surface static charges from which contaminants may not release. One possible solution is to change the electrical properties of the wire. However, attempts at decreasing toner build-up on the development wire by changing the electrical properties thereof, may result in an interference with the function of the wire and its ability to produce the formation of the toner powder cloud. Therefore, there is a specific need for electrode members which have a decreased tendency to accumulate toner and which also retain their electrical properties in order to prevent interference with the functioning thereof. There is an additional need for electrode members which have superior mechanical properties including durability against severe wear the electrode member receives when it is repeatedly brought into contact with tough rotating donor member surfaces.

#### SUMMARY OF THE INVENTION

Examples of objects of the present invention include:

It is an object of the present invention to provide an apparatus for reducing toner accumulation of electrode members in the development zone of a developing unit in an electrophotographic printing apparatus with many of the advantages indicated herein.

Another object of the present invention is to provide an apparatus for reducing toner adhesion to electrode members.

It is another object of the present invention to provide an apparatus comprising electrode members having a lower surface energy.

It is yet another object of the present invention to provide an apparatus comprising electrode members having increased mechanical strength.

Still yet another object of the present invention is to provide an apparatus comprising electrode members which have superior electrical properties.

A further object of the present invention is to provide an apparatus comprising electrode members which have smooth surfaces.

Many of the above objects have been met by the present invention, in embodiments, which includes: an apparatus for developing a latent image recorded on a surface, comprising: wire supports; a donor member spaced from the surface and being adapted to transport toner to a region opposed from the surface; an electrode member positioned in the space between the surface and the donor member, the electrode member being closely spaced from the donor member and being electrically biased to detach toner from the donor member thereby enabling the formation of a toner cloud in the space between the electrode member and the surface with detached toner from the toner cloud developing the latent image, wherein opposed end regions of the electrode member are attached to wire supports adapted to support the opposed end regions of said electrode member; and an inorganic coating on at least a portion of nonattached regions of said electrode member.

Embodiments further include: an electrophotographic process comprising: a) forming an electrostatic latent image on a charge-retentive surface; b) applying toner in the form of a toner cloud to said latent image to form a developed image on said charge retentive surface, wherein said toner is applied using a development apparatus comprising wire supports; a donor member spaced from the surface and being adapted to transport toner to a region opposed from the surface; an electrode member positioned in the space between the surface and said donor member, said electrode member being closely spaced from said donor member and being electrically biased to detach toner from said donor member thereby enabling the formation of a toner cloud in the space between said electrode member and the surface with detached toner from the toner cloud developing the latent image, wherein opposed end regions of said electrode member are attached to said wire supports adapted to support the opposed end regions of said electrode member; and an inorganic coating on at least a portion of nonattached regions of said electrode member.

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

5565

5570

5575

5580

5585

5590

5595

5600

5605

5610

<p

FIG. 5 is an illustration of wire contamination and wire history.

#### DETAILED DESCRIPTION

For a general understanding of the features of the present invention, a description thereof will be made with reference to the drawings.

FIG. 1 shows a development apparatus used in an electrophotographic printing machine such as that illustrated and described in U.S. Pat. No. 5,124,749, the disclosure of which is hereby incorporated by reference in its entirety. This patent describes the details of the main components of an electrophotographic printing machine and how these components interact. The present application will concentrate on the development unit of the electrophotographic printing machine. Specifically, after an electrostatic latent image has been recorded on a photoconductive surface, a photoreceptor belt advances the latent image to the development station. At the development station, a developer unit develops the latent image recorded on the photoconductive surface.

Referring now to FIG. 1, in a preferred embodiment of the invention, developer unit 38 develops the latent image recorded on the photoconductive surface 10. Preferably, developer unit 38 includes donor roller 40 and electrode member or members 42. Electrode members 42 are electrically biased relative to donor roll 40 to detach toner therefrom so as to form a toner powder cloud in the gap between the donor roll 40 and photoconductive surface 10. The latent image attracts toner particles from the toner powder cloud forming a toner powder image thereon. Donor roller 40 is mounted, at least partially, in the chamber of developer housing 44. The chamber in developer housing 44 stores a supply of developer material. The developer material is a two component developer material of at least carrier granules having toner particles adhering triboelectrically thereto. A magnetic roller 46 disposed interior of the chamber of housing 44 conveys the developer material to the donor roller 40. The magnetic roller 46 is electrically biased relative to the donor roller so that the toner particles are attracted from the magnetic roller to the donor roller.

More specifically, developer unit 38 includes a housing 44 defining a chamber 76 for storing a supply of two component (toner and carrier) developer material therein. Donor roller 40, electrode members 42 and magnetic roller 46 are mounted in chamber 76 of housing 44. The donor roller can be rotated in either the 'with' or 'against' direction relative to the direction of motion of belt 10. In FIG. 1, donor roller 40 is shown rotating in the direction of arrow 68. Similarly, the magnetic roller can be rotated in either the 'with' or 'against' direction relative to the direction of motion of belt 10. In FIG. 1, magnetic roller 46 is shown rotating in the direction of arrow 92. Donor roller 40 is preferably made from anodized aluminum or ceramic.

Developer unit 38 also has electrode members 42 which are disposed in the space between the belt 10 and donor roller 40. A pair of electrode members are shown extending in a direction substantially parallel to the longitudinal axis of the donor roller. The electrode members are made from of one or more thin (i.e., 50 to 100  $\mu\text{m}$  in diameter) stainless steel or tungsten electrode members which are closely spaced from donor roller 40. The distance between the electrode members and the donor roller is from about 5 to about 35  $\mu\text{m}$ , preferably about 10 to about 25  $\mu\text{m}$  or the thickness of the toner layer on the donor roll. The electrode members are self-spaced from the donor roller by the

thickness of the toner on the donor roller. To this end, the extremities of the electrode members supported by the tops of end bearing blocks also support the donor roller for rotation. The electrode member extremities are attached so that they are slightly above a tangent to the surface, including toner layer, of the donor structure. Mounting the electrode members in such a manner makes them insensitive to roll run-out due to their self-spacing.

As illustrated in FIG. 1, an alternating electrical bias is applied to the electrode members by an AC voltage source 78. The applied AC establishes an alternating electrostatic field between the electrode members and the donor roller is effective in detaching toner from the photoconductive member of the donor roller and forming a toner cloud about the electrode members, the height of the cloud being such as not to be substantially in contact with the belt 10. The magnitude of the AC voltage is relatively low and is in the order of 200 to 500 volts peak at a frequency ranging from about 9 kHz to about 15 kHz. A DC bias supply 80 which applies approximately 300 volts to donor roller 40 establishes an electrostatic field between photoconductive member of belt 10 and donor roller 40 for attracting the detached toner particles from the cloud surrounding the electrode members to the latent image recorded on the photoconductive member. At a spacing ranging from about 0.001  $\mu\text{m}$  to about 45  $\mu\text{m}$  between the electrode members and donor roller, an applied voltage of 200 to 500 volts produces a relatively large electrostatic field without risk of air breakdown. A cleaning blade 82 strips all of the toner from donor roller 40 after development so that magnetic roller 46 meters fresh toner to a clean donor roller. Magnetic roller 46 meters a constant quantity of toner having a substantially constant charge onto donor roller 40. This insures that the donor roller provides a constant amount of toner having a substantially constant charge in the development gap. In lieu of using a cleaning blade, the combination of donor roller spacing, i.e., spacing between the donor roller and the magnetic roller, the compressed pile height of the developer material on the magnetic roller, and the magnetic properties of the magnetic roller in conjunction with the use of a conductive, magnetic developer material achieves the deposition of a constant quantity of toner having a substantially charge on the donor roller. ADC bias supply 84 which applies approximately 100 volts to magnetic roller 46 establishes an electrostatic field between magnetic roller 46 and donor roller 40 so that an electrostatic field is established between the donor roller and the magnetic roller which causes toner particles to be attracted from the magnetic roller to the donor roller. Metering blade 86 is positioned closely adjacent to magnetic roller 46 to maintain the compressed pile height of the developer material on magnetic roller 46 at the desired level. Magnetic roller 46 includes a non-magnetic tubular member 88 made preferably from aluminum and having the exterior circumferential surface thereof roughened. An elongated magnet 90 is positioned interiorly of and spaced from the tubular member. The magnet is mounted stationarily. The tubular member rotates in the direction of arrow 92 to advance the developer material adhering thereto into the nip defined by donor roller 40 and magnetic roller 46. Toner particles are attracted from the carrier granules on the magnetic roller to the donor roller.

With continued reference to FIG. 1, an auger, indicated generally by the reference numeral 94, is located in chamber 76 of housing 44. Auger 94 is mounted rotatably in chamber 76 to mix and transport developer material. The auger has blades extending spirally outwardly from a shaft. The blades are designed to advance the developer material in the axial direction substantially parallel to the longitudinal axis of the shaft.

As successive electrostatic latent images are developed, the toner particles within the developer material are depleted. A toner dispenser (not shown) stores a supply of toner particles which may include toner and carrier particles. The toner dispenser is in communication with chamber 76 of housing 44. As the concentration of toner particles in the developer material is decreased, fresh toner particles are furnished to the developer material in the chamber from the toner dispenser. In an embodiment of the invention, the auger in the chamber of the housing mix the fresh toner particles with the remaining developer material so that the resultant developer material therein is substantially uniform with the concentration of toner particles being optimized. In this way, a substantially constant amount of toner particles are in the chamber of the developer housing with the toner particles having a constant charge. The developer material in the chamber of the developer housing is magnetic and may be electrically conductive. By way of example, in an embodiment of the invention wherein the toner includes carrier particles, the carrier granules include a ferromagnetic core having a thin layer of magnetite overcoated with a noncontinuous layer of resinous material. The toner particles may be made from a resinous material, such as a vinyl polymer, mixed with a coloring material, such as chromogen black. The developer material may comprise from about 90% to about 99% by weight of carrier and from 10% to about 1% by weight of toner. However, one skilled in the art will recognize that any other suitable developer material may be used.

In an alternative embodiment of the present invention, one component developer material consisting of toner without carrier may be used. In this configuration, the magnetic roller 46 is not present in the developer housing. This embodiment is described in more detail in U.S. Pat. No. 4,868,600, the disclosure of which is hereby incorporated by reference in its entirety.

An embodiment of the developer unit is further depicted in FIG. 2. The developer apparatus 34 comprises an electrode member 42 which is disposed in the space between the photoreceptor (not shown in FIG. 2) and the donor roll 40. The electrode 42 can be comprised of one or more thin (i.e., 50 to about 100  $\mu\text{m}$  in diameter) tungsten or stainless steel electrode members which are lightly positioned at or near the donor structure 40. The electrode member is closely spaced from the donor member. The distance between the wire(s) and the donor is approximately 0.001 to about 45  $\mu\text{m}$ , and preferably from about 10 to about 25  $\mu\text{m}$  or the thickness of the toner layer 43 on the donor roll. The wires as shown in FIG. 2 are self spaced from the donor structure by the thickness of the toner on the donor structure. The extremities or opposed end regions of the electrode member are supported by support members 54 which may also support the donor structure for rotation. In a preferred embodiment, the electrode member extremities or opposed end regions are attached so that they are slightly below a tangent to the surface, including toner layer, of the donor structure. Mounting the electrode members in such a manner makes them insensitive to roll runout due to their self-spacing.

In an alternative embodiment to that depicted in FIG. 1, the metering blade 86 is replaced by a combined metering and charging blade 86 as shown in FIG. 3. The combination metering and charging device may comprise any suitable device for depositing a monolayer of well charged toner onto the donor structure 40. For example, it may comprise an apparatus such as that described in U.S. Pat. No. 4,459,009, wherein the contact between weakly charged toner particles

and a triboelectrically active coating contained on a charging roller results in well charged toner. Other combination metering and charging devices may be employed, for example, a conventional magnetic brush used with two component developer could also be used for depositing the toner layer onto the donor structure, or a donor roller alone used with one component developer.

FIG. 4 depicts an enlarged view of a preferred embodiment of the electrode member of the present invention. Electrode wires 45 are positioned inside electrode member 42. The anchoring portions 55 of the electrode members are the portions of the electrode member which anchor the electrode member to the support member. The mounting sections 56 of the electrode member are the sections of the electrode members between the electrode member and the mounting means 54.

Toner particles are attracted to the electrode members primarily through electrostatic attraction. Toner particles adhere to the electrode members because the adhesion force of the toner is larger than the stripping force generated by the electric field of the electrode member. Generally, the adhesion force between a toner particle and an electrode member is represented by the general expression  $F_{ad}=q^2/kr^2+W$ , wherein  $F_{ad}$  is the force of adhesion,  $q$  is the charge on the toner particle,  $k$  is the effective dielectric constant of the toner and any dielectric coating, and  $r$  is the separation of the particle from its image charge within the wire which depends on the thickness, dielectric constant, and conductivity of the coating. Element  $W$  is the force of adhesion due to short range adhesion forces such as van der Waals and capillary forces. The force necessary to strip or remove particles from the electrode member is supplied by the electric field of the wire during half of its AC period,  $qE$ , plus effective forces resulting from mechanical motion of the electrode member and from bombardment of the wire by toner in the cloud. Since the adhesion force is quadratic in  $q$ , adhesion forces will be larger than stripping forces for sufficiently high values of  $q$ .

FIG. 5 contains an illustration of wire contamination and wire history. A photoreceptor 1 is positioned near wire 4 and contains an undeveloped image 6 which is subsequently developed by toner originating from donor member 3. Wire contamination occurs when fused toner 5 forms between the wire 4 and donor member 3. The problem is aggravated by toner fines and any toner components, such as high molecular weight, crosslinked and/or branched components, and the voltage breakdown between the wire member and the donor roll. Wire history is a change in developability due to toner 2 or toner components sticking to the top of the wire 4, the top of the wire being the part of the wire facing the photoreceptor.

In order to prevent the toner defects associated with wire contamination and wire history, the electrical properties of the electrode member can be changed, thereby changing the adhesion forces in relation to the stripping forces. However, such changes in the electrical properties of the electrode member may adversely affect the ability of the electrode member to adequately provide a toner cloud, which is essential for developing a latent image. The present invention is directed to an apparatus for reducing the unacceptable accumulation of toner on the electrode member while maintaining the desired electrical and mechanical properties of the electrode member. The electrode member of the present invention is coated with a material coating that reduces the significant attraction of toner particles to the electrode member which may result in toner accumulation. However, the material coating does not adversely interfere with the

mechanical or electrical properties of the electrode member. Materials having these qualities include materials with a low surface energy.

The low surface energy material decreases the accumulation of toner by assuring electrical continuity for charging the wires and eliminates the possibility of charge build-up. In addition, such low surface energy materials as described herein do not interfere with the electrical properties of the electrode member and do not adversely affect the electrode's ability to produce a toner powder cloud. Moreover, the electrode member maintains its tough mechanical properties, allowing the electrode member to remain durable against the severe wear the electrode member receives when it is repeatedly brought into contact with tough, rotating donor roll surfaces. Also, the electrode member maintains a "smooth" surface after the coating is applied. A smooth surface includes surfaces having a surface roughness of less than about 5 microns, preferably from about 0.01 to about 1 micron.

Examples of suitable low surface energy electrode coating materials include both organic materials and inorganic materials. It is preferred that the inorganic material possess the characteristics of low surface energy, high hardness, very low or no porosity, smooth surface characteristics, low friction and high wear resistance to enable the wire to withstand numerous cycling for every day use in an electrophotographic apparatus. Examples of suitable inorganic materials possessing the above characteristics include ceramics, borosilicate glasses, diamond and diamond like compounds, silicone hard coatings, molybdenum silicide, and derivatives thereof. Examples of ceramics having little or no porosity, include boron nitride, zirconium oxide, titanium carbide, silicon carbide, titanium nitride, zirconium diboride, yttrium oxide, glass ceramic (having about 75 percent by weight silica) and the like. Suitable ceramic coating materials are available as stable dispersions from ZYP Coatings Co. of Oak Ridge, Tenn. Heat resistant glass such as, for example, borosilicate glasses, are also suitable inorganic materials and possess the above characteristics. Glass coated wires are commercially available from AMTX Company of Canandagua, N.Y. and Pegasus of Springfield, Mass. Diamond and diamond derivative coatings including low grade diamonds such as, for example, bort and carbonado, are also suitable low surface inorganics and commercially available examples include "Dylyn Coating" by Advanced Refractory Technologies of Buffalo, N.Y. which is a self compensating interpenetrating network of carbon, hydrogen, silicone and oxygen. Another suitable low surface energy inorganic material is molybdenum disilicide ( $MoSi_2$ ) and its combination with silica, both forms of which are commercially available as stable dispersions from ZYP Coatings of Oak Ridge, Tenn. Other suitable low surface energy inorganic materials include hard silicone coatings such as, for example, silanes and siloxanes, which can be deposited on the wire surface by Ion Beam Assisted Deposition method, thereby forming inorganic hard silicone coatings. The details of this technique are published in the Journal of Materials Research, vol. 6, page 871, 1991, the disclosure of which is hereby incorporated by reference in its entirety.

A filler such as an electrically conductive filler, may be added to the material coating in the amount of from about 5 to about 35 percent by weight of total solids, preferably from about 15 to about 20 percent by weight of total solids. Total solids herein include the amount of filler and inorganic solid material, catalyst, and any additives. Examples of electrically conductive fillers include metal oxides such as tin

oxide, titanium oxide, zirconium oxide. Another preferred filler is carbon black, graphite or the like, with surface treatment of compounds such as for example, siloxane, silane, fluorine or the like. Specifically preferred treated carbon blacks include fluorinated carbons such as those described in co-pending U.S. patent application Ser. No. 08/635,356 filed Apr. 19, 1996, the disclosure of which is hereby incorporated by reference in its entirety.

The low surface energy inorganic coating material is preferably present in an amount of from about 5 to about 95 percent by weight of total solids, and preferably from about 10 to about 40 percent by weight of total solids. Total solids as used herein, refers to the total amount by weight of inorganic coating material, fillers, and additives contained in the coating solution.

The volume resistivity of the coated electrode is for example from about  $10^{-10}$  to about  $1^{-1}$  ohm-cm, and preferably from  $10^{-5}$  to  $10^{-1}$  ohm-cm. The surface roughness is less than about 5 microns and preferably from about 0.01 to about 1 micron.

In a preferred embodiment of the invention, the material coating is coated over at least a portion of the nonattached regions of the electrode member. The nonattached region of the electrode member is the entire outer surface region of the electrode minus the region where the electrode is attached to the mounting means 54 and minus the anchoring area (55 in FIG. 4). It is preferred that the coating cover the portion of the electrode member which is adjacent to the donor roll. In another preferred embodiment of the invention, the material coating is coated in an entire area of the electrode member located in a central portion of the electrode member and extending to an area adjacent to the nonattached portion of the electrode member. This area includes the entire surface of the electrode member minus the anchoring area (55 in FIG. 4). In an alternative embodiment, the entire length of the electrode member is coated with the material coating, including the anchoring area 55 and mounting area 56. In embodiments, at least a portion refers to the non-attached region being coated, or from about 10 to about 90 percent of the electrode member.

Toner can accumulate anywhere along the electrode member, but it will not adversely affect development unless it accumulates in the length of the electrode member near to the donor roll or on the length closest to the photoreceptor. Therefore, it is preferred that the material coating cover the electrode member along the entire length corresponding to the donor roll, and on the entire length corresponding to the photoreceptor.

The material coating may be deposited on at least a portion of the electrode member by any suitable, known method. These deposition methods include liquid and powder coating, dip and spray coating, and ion beam assisted and RF plasma deposition. In a preferred deposition method, the material coating is coated on the electrode member by dip coating. With silicone materials, it is preferred to apply these coatings by ion beam assisted deposition. After coating, the inorganic coating is preferably air dried and cured at a temperature suitable for curing the specific inorganic material. Curing temperatures range from about 400 to about 1400° C., and preferably from about 600 to about 1200° C.

The average thickness of the coating is from about 1 to about 30  $\mu m$  thick, and preferably from about 2 to about 10  $\mu m$  thick. If the coating is applied to only a portion of the electrode member, the thickness of the coating may or may not taper off at points farthest from the midpoint of the electrode member. Therefore, the thickness of the coating may decrease at points farther away from the midpoint of the electrode.

## 11

The electrode members of the present invention, the embodiments of which have been described herein exhibit superior performance in terms wear resistance and decreased accumulation of toner on the surface of the electrode member, while also maintaining electrical properties which stimulate production of powder cloud development without charge build-up. In addition, the electrode members herein exhibit superior mechanical properties such as durability against donor roll surfaces which are normally made of tough materials such as ceramics.

All the patents and applications referred to herein are hereby specifically, and totally incorporated herein by reference in their entirety in the instant specification.

The following Examples further define and describe embodiments of the present invention. Unless otherwise indicated, all parts and percentages are by weight.

## EXAMPLES

## Example 1

## Preparation of Wire to be Coated

A stainless steel wire of about 3 mil thickness is preferably cleaned to remove obvious contaminants.

A dip coating apparatus with a 1 inch (diameter) by 15 inches (length) glass cylinder sealed at one end to hold the liquid coating material can be used for dip coating the wire. A cable attached to a Bodine Electric Company type NSH-12R motor is used to raise and lower a wire support holder that keeps the wire taut during the coating process. The dip and withdraw rate of the wire holder into and out of the coating solution can be regulated by a motor control device from B&B Motors & Control Corporation, (NOVA PD DC motor speed control). After coating, a motor driven device is used to twirl the wire around its axis while it receives external heating to allow for controlled solvent evaporation. When the coating is dry and/or non-flowable, the coated wire can be heated in a flow through oven using a time and temperature schedule to complete either drying or cure/post cure of the coating.

The general procedure may include: (A) cleaning and degreasing the wire with an appropriate solvent, for example, acetone, alcohol or water, and roughened if necessary by, for example, sand paper; (B) the coating material may be adjusted to the proper viscosity and solids content by adding solids or solvent to the solution; and (C) the wire is dipped into and withdrawn from the coating solution, dried and cured/post cured, if necessary, and dipped again, if required. The coating thickness and uniformity are a function of withdrawal rate and solution viscosity, (solids content in most solvent based systems) and a drying schedule consistent with the uniform solidification of the coating.

## EXAMPLES

## Preparation of Inorganic Coating Solutions

## Example 1

A stainless steel wire of 3 mil thickness can be cleaned to remove obvious contaminants. High purity titanium nitride (TiN) dispersion Type "TN" obtained from ZYP Coatings Inc., of Oak Ridge, Tenn., having 75% solids content is then added to the coating tank of the dip coater. This coating can be applied using conventional dip coating method as described in Example 1. The coatings can then be air dried and cured at 400° C. for 12 hours. The resulting coating

## 12

surface can then be hand polished through a rubbing action by using a back and forth wiping motion.

## Example 2

5 A dispersion containing zirconium diboride obtained from ZYP Coatings Inc, of Oak Ridge, Tenn. as Type "ZB-MOD" having 58% solids contents can be used as an inorganic coating solution. This coating can be applied using conventional dip coating method as described in Example 1. The coatings can then be air dried and cured at 1,200°–1,600° C.

## Example 3

10 15 A dispersion of molybdenum disilicide obtained from ZYP Coatings Inc, of Oak Ridge, Tenn. sold as Type "MS" having about 50% solids can be used as an inorganic coating. This coating can be applied using conventional dip coating method as described in Example 1. The coatings can then be air dried and cured at 1,200°–1,600° C.

## Example 4

20 25 A dispersion of boron nitride obtained from ZYP Coatings Inc, of Oak Ridge, Tenn. sold as Type "BN-MOD" and having about 25% solids can be used as an inorganic coating. This coating can be applied using conventional dip coating method as described in Example 1. The coatings can then be air dried and cured at 700°–1,000° C.

## Example 5

30 35 A dispersion of titanium carbide obtained from ZYP Coatings Inc, of Oak Ridge, Tenn. sold as Type "T" and having about 45% solids can be used as an inorganic coating. This coating can be applied using conventional dip coating method as described in Example 1. The coatings can then be air dried and cured at 700°–900° C.

## Example 6

40 45 A steel wire can be coated by Advanced Refractory Technology of Buffalo, N.Y. with self compensating interpenetrating network of carbon, hydrogen, silicone and oxygen which is commercially called "Dylyn". The thickness of the coating is estimated to be from about 1 to about 3 microns, very smooth and relatively hard. The electrical conductivity is estimated to be about  $10^{-9}$  ohm-cm.

50 While the invention has been described in detail with reference to specific and preferred embodiments, it will be appreciated that various modifications and variations will be apparent to the artisan. All such modifications and embodiments as may readily occur to one skilled in the art are intended to be within the scope of the appended claims.

What is claimed is:

1. An apparatus for developing a latent image recorded on a surface, comprising:  
55 wire supports;  
a donor member spaced from the surface and being adapted to transport toner to a region opposed from the surface;  
an electrode member positioned in the space between the surface and the donor member, the electrode member being closely spaced from the donor member and being electrically biased to detach toner from the donor member thereby enabling the formation of a toner cloud in the space between the electrode member and the surface with detached toner from the toner cloud developing the latent image, wherein opposed end

## 13

- regions of the electrode member are attached to wire supports adapted to support the opposed end regions of said electrode member; and
- 5 a low surface energy inorganic material coating on at least a portion of nonattached regions of said electrode member.
2. An apparatus in accordance with claim 1, wherein said low surface energy of said low surface energy material is from about 10 to about 25 dynes/cm.
- 10 3. An apparatus in accordance with claim 2, wherein said inorganic coating is borosilicate glass.
4. An apparatus in accordance with claim 2, wherein said inorganic coating is selected from the group consisting of diamond and diamond derivatives.
- 15 5. An apparatus in accordance with claim 2, wherein said inorganic coating is molybdenum silicide.
6. An apparatus in accordance with claim 1, wherein said inorganic coating comprises a material selected from the group consisting of ceramics, borosilicate glass, diamond, MoS<sub>2</sub> and derivatives thereof.
- 20 7. An apparatus in accordance with claim 6, wherein said inorganic coating is a ceramic material selected from the group consisting of boron nitride, zirconium oxide, titanium carbide, silicon carbide, titanium nitride, zirconium diboride, and yttrium oxide.
- 25 8. An apparatus in accordance with claim 1, wherein said inorganic coating comprises an electrically conductive filler dispersed therein.
9. An apparatus in accordance with claim 8, wherein said electrically conductive filler is selected from the group consisting of carbon black, metal oxides, and metal hydroxides.
- 30 10. An apparatus in accordance with claim 9, wherein said conductive metal filler is selected from the group consisting of tin oxide, titanium oxide, zirconium oxide, calcium hydroxide, and magnesium hydroxide.
- 35 11. An apparatus in accordance with claim 9, wherein said electrically conductive filler is carbon black.
12. An apparatus in accordance with claim 1, wherein said inorganic coating is present on from about 10 to about 90 percent of said electrode member.
- 40 13. An apparatus in accordance with claim 1, wherein said inorganic coating is of a thickness of from about 1  $\mu\text{m}$  to about 5  $\mu\text{m}$ .
14. An apparatus in accordance with claim 1, wherein said electrode member includes more than one thin diameter wires.
- 45 15. An apparatus in accordance with claim 1, wherein said thin diameter wires have a diameter of from about 50 to about 100  $\mu\text{m}$ .
16. An apparatus in accordance with claim 1, wherein said donor member is closely spaced from said donor member a distance of from about 0.001 to about 45  $\mu\text{m}$ .
- 50 17. An apparatus in accordance with claim 1, wherein said inorganic coating material is coated on said electrode wire by dip coating.
- 55

## 14

18. An apparatus in accordance with claim 17, wherein said dip coated inorganic coating material is cured at a temperature of from about 400 to about 1,400° C.
19. An electrophotographic process comprising:
- forming an electrostatic latent image on a charge-retentive surface;
  - applying toner in the form of a toner cloud to said latent image to form a developed image on said charge retentive surface, wherein said toner is applied using a development apparatus comprising wire supports; a donor member spaced from the surface and being adapted to transport toner to a region opposed from the surface; an electrode member positioned in the space between the surface and said donor member, said electrode member being closely spaced from said donor member and being electrically biased to detach toner from said donor member thereby enabling the formation of a toner cloud in the space between said electrode member and the surface with detached toner from the toner cloud developing the latent image, wherein opposed end regions of said electrode member are attached to said wire supports adapted to support the opposed end regions of said electrode member; and a low surface energy inorganic coating on at least a portion of nonattached regions of said electrode member;
  - transferring the toner image from said charge-retentive surface to a substrate; and
  - fixing said toner image to said substrate.
20. An apparatus for developing a latent image recorded on a surface, comprising:
- wire supports;
- a donor member spaced from the surface and being adapted to transport toner to a region opposed from the surface;
- an electrode member positioned in the space between the surface and the donor member, the electrode member being closely spaced from the donor member and being electrically biased to detach toner from the donor member thereby enabling the formation of a toner cloud in the space between the electrode member and the surface with detached toner from the toner cloud developing the latent image, wherein opposed end regions of the electrode member are attached to wire supports adapted to support the opposed end regions of said electrode member; and
- a low energy surface inorganic material coating on at least a portion of nonattached regions of said electrode member, wherein said low surface energy material has a low surface energy of from about 10 to about 25 dynes/cm.

\* \* \* \* \*

UNITED STATES PATENT AND TRADEMARK OFFICE  
**CERTIFICATE OF CORRECTION**

PATENT NO. : 5,805,964

DATED : 9/8/98

INVENTOR(S) : Badesha et al.

It is certified that error appears in the above-identified patent and that said Letters Patent is hereby corrected as shown below:

Column 14, line 50, delete "low energy surface" and replace with --low surface energy--.

Signed and Sealed this

Twenty-third Day of February, 1999

Attest:



Q. TODD DICKINSON

Attesting Officer

Acting Commissioner of Patents and Trademarks